

STEPHEN M. ALLEN, OF WOBURN, MASSACHUSETTS.

Letters Patent No. 80,048, dated July 21, 1868.

## IMPROVED ARTIFICIAL-LEATHER BELTING.

The Schedule referred to in these Letters Patent and making part of the same.

## TO WHOM IT MAY CONCERN:

Be it known that I, STEPHEN M. ALLEN, of Woburn, in the county of Middlesex, and State of Massachusetts, have invented a new and improved Artificial-Leather Belting; and I hereby declare the following to be a full, clear, and exact description of the same.

In the practical use of my artificial-leather belting, heretofore patented by me, I have found many useful and important ways in which to apply it.

I will now describe my new process and its application.

I make sheets of pulped leather paper, made from tanned and untanned hides, or either of them, or other animal tissues, in combination with vegetable fibre, gelatinous and resinous substances, and sometimes bullock's blood, made substantially as described in two Letters Patent taken out by me heretofore, for the manufacture of artificial-leather belting, and prepare the same in a proper manner, of different widths and thicknesses, according to circumstances. I then set these sheets together, to any desired thickness and width, with some flexible cementing-compound which shall hold them firmly together, and, if need be, rivet or sew them. Sometimes I use other substances between or on one or both sides of these sheets, set together, such as canvas, cloth, twine, strips of iron, wood, or common leather. Sometimes I use the artificial leather upon the inside or outside (as may be desired) of common leather or other belting, to render it more firm and less liable to stretch, as well as to equalize the thickness and protect the laps or joints from wear and accident.

The advantages of these improvements are, that, in setting together a number of sheets of the artificial-leather or paper belting to form the thickness of the belt, the belt is made stronger than if made of great thickness in one sheet. The cementing-compound between the sheets prevents, to a great degree, the absorption of moisture, and renders the belt less porous, whereby a more perfect vacuum is formed between the belt and pulley. When the artificial leather is used in combination with common leather, or with any or all of the other substances named, it will, when joined or cemented together as described, by its adaptability, hold them in better condition and more solid and less elastic than they otherwise could be. For instance, by taking a piece of common belting-leather, which is unequal in thickness and texture, and not strong enough for the purpose needed, and setting it to one or more thicknesses of the artificial leather properly cemented and secured, its strength and firmness are greatly increased, and it will run better and truer than it otherwise could.

Having now described my invention, and the manner in which the same is or may be carried into effect, what I claim, and desire to secure by Letters Patent, is as follows:

1. I claim the attaching, cementing, gluing, stitching, or uniting together of sheets for artificial-leather belting or banding made from pulped animal fibre, tanned or untanned, used alone or in combination with other vegetable fibre, or with other further combination with resinous or gelatinous substances.
2. I claim attaching, cementing, gluing, riveting, or stitching sheets or strips of artificial-leather paper for belting, made from pulped animal fibre, tanned or untanned, alone or mixed in further combination with other pulped vegetable fibre, to sheets of common leather for belting, whether the sheets of leather are laid upon either one or both sides, or between sheets of artificial leather.
3. I claim the combination of sheets of artificial leather for belting, with sheets of leather, canvas, cloth, wood, yarn, iron, or wire, when properly attached together for the purpose, by gluing, cementing, riveting, or stitching the same.
4. I claim the overlapping and strengthening of joints in leather, artificial leather, or other belting, by the use of artificial-leather sheets, set on and over the laps or joints in belting, by cementing, gluing, riveting, or stitching the same, substantially as herein described.
5. I claim a belting made of pulped artificial leather, as described, by combining sheets made of the same to the other substances named, or any of them, as described, such as leather, canvas, cloth, wood, yarn, iron, or wire, properly set together in the manner and for the purposes substantially as described.
6. I claim the application of artificial-leather paper to veneer and increase the thickness and strength of leather belting by applying the same to the softer and thinner parts of leather belting, making them of uniform thickness, and nearly non-elastic, either when applied outside or between strips of leather, and confined substantially as herein described.

In testimony whereof, I have signed my name to this specification before two subscribing witnesses.

STEPHEN M. ALLEN.

Witnesses:

THOS. S. RIDGWAY,  
L. BURNETT.